



US011008529B2

(12) **United States Patent**  
**Jakupca et al.**

(10) **Patent No.:** **US 11,008,529 B2**  
(45) **Date of Patent:** **May 18, 2021**

(54) **POLYMERIC POLY-PHOSPHORUS ADDITIVES FOR: GEAR OIL, GREASE, ENGINE-OIL, COMBUSTION-ENGINE LUBRICANT, AUTOMATIC TRANSMISSION FLUID, ANTI-WEAR AGENTS, TWO-CYCLE ENGINE LUBRICANT, OR MARINE-ENGINE LUBRICANT**

(71) Applicant: **Dover Chemical Corporation**, Dover, OH (US)

(72) Inventors: **Michael Jakupca**, Canton, OH (US); **Jacob Weingart**, Canton, OH (US); **Ben Rohr**, Bolivar, OH (US)

(73) Assignee: **Dover Chemical Corporation**, Dover, OH (US)

(\*) Notice: Subject to any disclaimer, the term of this patent is extended or adjusted under 35 U.S.C. 154(b) by 0 days.

(21) Appl. No.: **16/713,993**

(22) Filed: **Dec. 13, 2019**

(65) **Prior Publication Data**

US 2020/0231893 A1 Jul. 23, 2020

**Related U.S. Application Data**

(60) Provisional application No. 62/779,219, filed on Dec. 13, 2018.

(51) **Int. Cl.**

**C10M 137/02** (2006.01)  
**C10M 153/04** (2006.01)

(Continued)

(52) **U.S. Cl.**

CPC ..... **C10M 153/04** (2013.01); **C10M 137/02** (2013.01); **C10M 137/04** (2013.01);

(Continued)

(58) **Field of Classification Search**  
CPC ..... C10M 153/04; C10M 137/04;  
C10M 137/02; C10M 137/105; C10M  
2223/049;  
(Continued)

(56) **References Cited**

**U.S. PATENT DOCUMENTS**

6,489,271 B1 12/2002 Richardson  
2010/0137174 A1 \* 6/2010 Maeda ..... C10M 133/44  
508/279

(Continued)

**FOREIGN PATENT DOCUMENTS**

EP 3006448 A1 4/2016  
JP S5090581 A 12/1973  
(Continued)

**OTHER PUBLICATIONS**

XP-002780520 (Synthesis and hydrolytic stability of polyoxyethylene-H-phosphonates) (Year: 2008).\*

(Continued)

*Primary Examiner* — Taiwo Oladapo

(74) *Attorney, Agent, or Firm* — Schlue IP Law; Daniel J. Schlue

(57) **ABSTRACT**

A method having the step of using a compound as an additive for: gear oil, grease, engine oil, combustion-engine lubricant, automatic transmission fluid, two-cycle engine lubricant, marine-engine lubricant, or anti-wear agent, the compound having the structure:



(Continued)



wherein each R is an independently selected alkylphenol-free moiety that is a C<sub>1-22</sub> alkyl, C<sub>6-40</sub> cycloalkyl, C<sub>3-20</sub> methoxy alkyl glycol ether, C<sub>3-20</sub> alkyl glycol ether, or Y—OH moiety; wherein each Y is an independently selected alkylphenol-free moiety that is a C<sub>2-40</sub> alkylene, C<sub>6-40</sub> cycloalkylene, C<sub>2-20</sub> alkylene glycol ether, or C<sub>3-40</sub> alkylene lactone moiety; wherein each m is an independently selected integer ranging from 1 to 100; and wherein x is an integer ranging from 1 to 1000.

### 34 Claims, 3 Drawing Sheets

(51) **Int. Cl.**

**C10M 137/04** (2006.01)  
**C10M 137/10** (2006.01)  
**C10N 40/25** (2006.01)  
**C10N 40/04** (2006.01)

(52) **U.S. Cl.**

CPC .... **C10M 137/105** (2013.01); **C10M 2223/04** (2013.01); **C10M 2223/047** (2013.01); **C10M 2223/049** (2013.01); **C10M 2225/00** (2013.01); **C10N 2040/04** (2013.01); **C10N 2040/042** (2020.05); **C10N 2040/25** (2013.01); **C10N 2040/252** (2020.05)

(58) **Field of Classification Search**

CPC ..... C10M 2225/00; C10M 2223/047; C10M 2223/04; C10N 2040/252; C10N 2040/042; C10N 2040/25; C10N 2040/04

See application file for complete search history.

(56)

### References Cited

#### U.S. PATENT DOCUMENTS

|              |     |         |         |       |             |  |
|--------------|-----|---------|---------|-------|-------------|--|
| 2011/0306530 | A1* | 12/2011 | Manabe  | ..... | C10M 137/04 |  |
|              |     |         |         |       | 508/287     |  |
| 2013/0079264 | A1  | 3/2013  | Tipton  | ..... |             |  |
| 2014/0329943 | A1* | 11/2014 | Jakupca | ..... | C08G 79/04  |  |
|              |     |         |         |       | 524/128     |  |

#### FOREIGN PATENT DOCUMENTS

|    |               |      |        |       |              |  |
|----|---------------|------|--------|-------|--------------|--|
| JP | 2016074657    | A    | 5/2016 |       |              |  |
| WO | 2016077134    | A1   | 5/2016 |       |              |  |
| WO | WO-2016077134 | A1 * | 5/2016 | ..... | C10M 159/123 |  |

### OTHER PUBLICATIONS

Database CA [Online] Chemical Abstracts Services, Columbus, Ohio, US, Noda, Ippei, et al.: "Lubricants for synthetic fibers", XP002780518 retrieved from STN Database accession No. 1986:150749—abstract; 2 pages.

Database CA [Online] Chemical Abstracts Services, Columbus, Ohio, US, Nobis, Markus N., et al.: "Poly (arylazophosphonate)s new arylazophosphonate-containing monomers for synthesis of laser-structurable polymers", XP002780519 retrieved from STN Database accession No. 2001:735270—abstract; and Macromolecular Chemistry and Physics, 202 (13), 2769-2775 Coden: Mchps; ISSN: 1022-1352, 2001, DOI: 10.1002/1521-3935 (Sep. 1, 2001) 202:13<2769: 2 pages.

Database CA [Online] Chemical Abstracts Services, Columbus, Ohio, US, Gitsov, Ivan et al.: "Synthesis and hydrolytic stability of poly(oxyethylene-H-phosphonate)s", XP002780520 retrieved from STN Database accession No. 2008:724200 abstract; and Journal of Polymer Science, Part A: Polymer Chemistry, 46(12), 4130-4139 CODEN: JPACES; ISSN: 0887-624X, 2008, DOI: 10.1002/POLA. 22759 10.1002/POLA.22759; 2 pages.

Database CA [Online] Chemical Abstracts Services, Columbus, Ohio, US, Keglevich, Gyorgy, et al.: "Microwave-assisted alcholysis of dialkyl phosphites by ethylene glycol and ethanolamine", XP002780521 retrieved from STN Database accession No. 2014:1930090 abstract; and Pure and Applied Chemistry, 86(11), 1723-1728 CODEN: PACHAS; ISSN: 0033-4545, 2014, DOI: 10.1515/PAC-2014-0601 10.1515/PAC-2014-0601; 1 page.

Database CA [Online] Chemical Abstracts Services, Columbus, Ohio, US, Han, Hengwen, et al.: "Biphosphite amine salt and its preparing method, application thereof and lubricating oil composition", XP002780522 retrieved from STN Database accession No. 2014:2007198 abstract; 2 pages.

Database CA [Online] Chemical Abstracts Services, Columbus, Ohio, US, Tominaga, Eiji, et al.: "Lubricating oil compositions for sliding guideway", XP002780523 retrieved from STN Database accession No. 1996:641045 abstract & JP H08 209175 A (Nippon Oil Co Ltd) Aug. 13, 1996 (Aug. 13, 1996); 1 page.

International Search Report for corresponding PCT application; 14 pages.

www.mdpi.com/journal/lubricants, David W. Johnson, et al.: "Phosphate Esters, Thiophosphates Esters and Metal Thiophosphates as Lubricant Additives" Published Dec. 18, 2013, 132-148, ISSN 2075-4442, DOI: 10.3390/lubricants 1040132: 17 pages.

Ciba IRGALUBE TPPT Extreme Pressure/antiwear additive, Ciba Speciality Chemicals, Inc, Reference AD7, CH-4002 Basle, Publ. No. 28979/96/e, Edited in Switzerland; 8 pages.

Extreme Pressure/Antiwear Additive Ciba IRGALUBE 211cd, Alkylated triphenyl phosphorothionate; 1 page.

Dover Chemical Corporation, Doverlube SP-44, Light Colored Sulphur-Phosphorus Additive; 1 page.

\* cited by examiner



Figure 1



Figure 2



Figure 3



Figure 4



Figure 5

1

**POLYMERIC POLY-PHOSPHORUS  
ADDITIVES FOR: GEAR OIL, GREASE,  
ENGINE-OIL, COMBUSTION-ENGINE  
LUBRICANT, AUTOMATIC TRANSMISSION  
FLUID, ANTI-WEAR AGENTS, TWO-CYCLE  
ENGINE LUBRICANT, OR MARINE-ENGINE  
LUBRICANT**

**CROSS-REFERENCE TO RELATED  
APPLICATIONS**

This patent application claims priority to U.S. provisional patent application 62/779,219 having a filing date of Dec. 13, 2018. The subject matter of U.S. provisional patent application 62/779,219 is hereby incorporated by reference in its entirety.

**BACKGROUND OF THE INVENTION**

The following are all known: gear oils, greases, engine-oil additives, combustion-engine lubricants, automatic transmission fluids, anti-wear agents, two-cycle engine lubricants, and marine-engine lubricants. With all of them, there is a need for improved performance.

**BRIEF SUMMARY OF THE INVENTION**

A method having the step of using a compound as an additive for: gear oil, grease, engine oil, combustion-engine lubricant, automatic transmission fluid, two-cycle engine lubricant, marine-engine lubricant, or anti-wear agent, the compound having the structure:



wherein each R is an independently selected alkylphenol-free moiety that is a  $C_{1-22}$  alkyl,  $C_{6-40}$  cycloalkyl,  $C_{3-20}$  methoxy alkyl glycol ether,  $C_{3-20}$  alkyl glycol ether, or Y—OH moiety; wherein each Y is an independently selected alkylphenol-free moiety that is a  $C_{2-40}$  alkylene,  $C_{6-40}$  cycloalkylene,  $C_{2-20}$  alkylene glycol ether, or  $C_{3-40}$  alkylene lactone moiety; wherein each m is an independently selected integer ranging from 1 to 100; and wherein x is an integer ranging from 1 to 1000.

A method having the step of using a compound as an additive for: gear oil, grease, engine oil, combustion-engine lubricant, automatic transmission fluid, two-cycle engine lubricant, marine-engine lubricant, or anti-wear agent, the compound having the structure:



wherein each R is an independently selected alkylphenol-free moiety that is a  $C_{1-22}$  alkyl,  $C_{6-40}$  cycloalkyl,  $C_{3-20}$  methoxy alkyl glycol ether,  $C_{3-20}$  alkyl glycol ether, or

2

Y—OH moiety; wherein each Y is an independently selected alkylphenol-free moiety that is a  $C_{2-40}$  alkylene,  $C_{6-40}$  cycloalkylene,  $C_{2-20}$  alkylene glycol ether, or  $C_{3-40}$  alkylene lactone moiety; wherein each m is an independently selected integer ranging from 2 to 100; and wherein x is an integer ranging from 1 to 1000.

A method having the step of using a compound as an additive for: gear oil, grease, engine oil, combustion-engine lubricant, automatic transmission fluid, two-cycle engine lubricant, marine-engine lubricant, or anti-wear agent, the compound having the structure:



wherein each R is an independently selected alkylphenol-free moiety that is a  $C_{1-22}$  alkyl,  $C_{6-40}$  cycloalkyl,  $C_{3-20}$  methoxy alkyl glycol ether,  $C_{3-20}$  alkyl glycol ether, or Y—OH moiety; wherein each Y is an independently selected alkylphenol-free moiety that is a  $C_{2-40}$  alkylene,  $C_{6-40}$  cycloalkylene,  $C_{2-20}$  alkylene glycol ether, or  $C_{3-40}$  alkylene lactone moiety; wherein each m is an independently selected integer ranging from 2 to 100; and wherein x is an integer ranging from 1 to 1000.

A method having the step of using a compound as an additive for: gear oil, grease, engine oil, combustion-engine lubricant, automatic transmission fluid, two-cycle engine lubricant, marine-engine lubricant, or anti-wear agent, the compound having the structure:



wherein each R is an independently selected alkylphenol-free moiety that is a  $C_{1-22}$  alkyl,  $C_{6-40}$  cycloalkyl,  $C_{3-20}$  methoxy alkyl glycol ether,  $C_{3-20}$  alkyl glycol ether, or Y—OH moiety; wherein each Y is an independently selected alkylphenol-free moiety that is a  $C_{2-40}$  alkylene,  $C_{6-40}$  cycloalkylene,  $C_{2-20}$  alkylene glycol ether, or  $C_{3-40}$  alkylene lactone moiety; wherein each m is an independently selected integer ranging from 2 to 100; wherein each Z is independently selected from the group consisting of S and O; and wherein x is an integer ranging from 1 to 1000.

A method having the step of using a copolymer compound as an additive for: gear oil, grease, engine oil, combustion-engine lubricant, automatic transmission fluid, two-cycle engine lubricant, marine-engine lubricant, or anti-wear agent, the compound having the structure:



wherein each R is an independently selected alkylphenol-free moiety that is a  $C_{1-22}$  alkyl,  $C_{6-40}$  cycloalkyl,  $C_{3-20}$  methoxy alkyl glycol ether,  $C_{3-20}$  alkyl glycol ether, or Y—OH moiety; wherein each Y is an independently selected alkylphenol-free moiety that is a  $C_{2-40}$  alkylene,  $C_{6-40}$  cycloalkylene,  $C_{2-20}$  alkylene glycol ether, or  $C_{3-40}$  alkylene lactone moiety; wherein  $Y_1$  and  $Y_2$  are different; wherein each m is an independently selected integer ranging from 1 to 100; wherein each Z is independently selected from the group consisting of S, H, O, and nothing; and wherein each x is an independently selected integer ranging from 1 to 1000.

A method having the step of using a compound as an additive for: gear oil, grease, engine oil, combustion-engine lubricant, automatic transmission fluid, two-cycle engine lubricant, marine-engine lubricant, or anti-wear agent, the compound having the structure:



wherein each R is an independently selected alkylphenol-free moiety that is a  $C_{1-22}$  alkyl,  $C_{6-40}$  cycloalkyl,  $C_{3-20}$  methoxy alkyl glycol ether,  $C_{3-20}$  alkyl glycol ether, or Y—OH moiety; wherein each Y is an independently selected alkylphenol-free moiety that is a  $C_{2-40}$  alkylene,  $C_{6-40}$  cycloalkylene,  $C_{2-20}$  alkylene glycol ether, or  $C_{3-40}$  alkylene lactone moiety; wherein each m is an independently selected integer ranging from 1 to 100; and wherein x is an integer ranging from 1 to 1000.

#### BRIEF DESCRIPTION OF THE SEVERAL VIEWS OF THE DRAWING

FIG. 1 is a picture of a Timken testing apparatus.

FIG. 2 is a graph showing Falex Pin and Vee Block test results.

FIG. 3 is a graph showing Falex Pin and Vee Block test results.

FIG. 4 is a graph showing Falex Pin and Vee Block test results.

FIG. 5 is a graph showing Falex Pin and Vee Block test results.

#### DETAILED DESCRIPTION OF THE INVENTION

Embodiments are directed to compounds that are useful as additives for: gear oil, grease, engine-oil, combustion-engine lubricant, automatic transmission fluid, two-cycle engine lubricant, and marine-engine lubricant. The compounds are also useful as an anti-wear additive or anti-wear agent.

An embodiment is directed to polyhydrogen-phosphite compounds having the general structure:



wherein each R is an independently selected alkylphenol-free moiety that is a  $C_{1-22}$  alkyl,  $C_{6-40}$  cycloalkyl,  $C_{3-20}$  methoxy alkyl glycol ether,  $C_{3-20}$  alkyl glycol ether, or Y—OH moiety;

wherein each Y is an independently selected alkylphenol-free moiety that is a  $C_{2-40}$  alkylene,  $C_{6-40}$  cycloalkylene,  $C_{2-20}$  alkylene glycol ether, or  $C_{3-40}$  alkylene lactone moiety;

wherein each m is an independently selected integer ranging from 1 to 100; and

wherein x is an integer ranging from 1 to 1000.

In some polyhydrogen-phosphite embodiments, each Y is an independently selected ethylene, propylene, cyclohexene dimethanol, or caprylene lactone moiety.

In some polyhydrogen-phosphite embodiments, the compound has a weight ranging from 1000 to 30000 Daltons. In some polyhydrogen-phosphite embodiments, the compound has a weight ranging from 400 to 30000 Daltons. In some polyhydrogen-phosphite embodiments, the compound has a weight ranging from 500 to 30000 Daltons.

An embodiment is directed to phosphate compounds having the general structure:



wherein each R is an independently selected alkylphenol-free moiety that is a  $C_{1-22}$  alkyl,  $C_{6-40}$  cycloalkyl,  $C_{3-20}$  methoxy alkyl glycol ether,  $C_{3-20}$  alkyl glycol ether, or Y—OH moiety;

wherein each Y is an independently selected alkylphenol-free moiety that is a  $C_{2-40}$  alkylene,  $C_{6-40}$  cycloalkylene,  $C_{2-20}$  alkylene glycol ether, or  $C_{3-40}$  alkylene lactone moiety;

wherein each m is an independently selected integer ranging from 1 to 100; and

wherein x is an integer ranging from 1 to 1000.

In some phosphate embodiments, each Y is an independently selected ethylene, propylene, cyclohexene dimethanol, or caprylene lactone moiety.

In some phosphate embodiments, the compound has a weight ranging from 1000 to 30000 Daltons. In some phosphate embodiments, the compound has a weight ranging from 400 to 30000 Daltons. In some phosphate embodiments, the compound has a weight ranging from 500 to 30000 Daltons.

An embodiment is directed to thiophosphate compounds having the general structure:



wherein each R is an independently selected alkylphenol-free moiety that is a  $C_{1-22}$  alkyl,  $C_{6-40}$  cycloalkyl,  $C_{3-20}$  methoxy alkyl glycol ether,  $C_{3-20}$  alkyl glycol ether, or Y—OH moiety;

wherein each Y is an independently selected alkylphenol-free moiety that is a  $C_{2-40}$  alkylene,  $C_{6-40}$  cycloalkylene,  $C_{2-20}$  alkylene glycol ether, or  $C_{3-40}$  alkylene lactone moiety;

wherein each m is an independently selected integer ranging from 1 to 100; and

wherein x is an integer ranging from 1 to 1000.

In some thiophosphate embodiments, each Y is an independently selected ethylene, propylene, cyclohexene dimethanol, or caprylene lactone moiety.

In some thiophosphate embodiments, the compound has a weight ranging from 1000 to 30000 Daltons. In some thiophosphate embodiments, the compound has a weight ranging from 400 to 30000 Daltons. In some thiophosphate embodiments, the compound has a weight ranging from 500 to 30000 Daltons.

An embodiment is directed to phosphorus-containing compounds having the general structure:



wherein each R is an independently selected alkylphenol-free moiety that is a  $C_{1-22}$  alkyl,  $C_{6-40}$  cycloalkyl,  $C_{3-20}$  methoxy alkyl glycol ether,  $C_{3-20}$  alkyl glycol ether, or Y—OH moiety;

wherein each Y is an independently selected alkylphenol-free moiety that is a  $C_{2-40}$  alkylene,  $C_{6-40}$  cycloalkylene,  $C_{2-20}$  alkylene glycol ether, or  $C_{3-40}$  alkylene lactone moiety;

wherein each m is an independently selected integer ranging from 1 to 100;

wherein each Z is independently selected from the group consisting of S and O; and

wherein x is an integer ranging from 1 to 1000.

In some phosphorus-containing embodiments, each Y is an independently selected ethylene, propylene, cyclohexene dimethanol, or caprylene lactone moiety.

In some phosphorus-containing-compound embodiments, the compound has a weight ranging from 1000 to 30000 Daltons. In some phosphorus-containing embodiments, the compound has a weight ranging from 400 to 30000 Daltons. In some phosphorus-containing embodiments, the compound has a weight ranging from 500 to 30000 Daltons.

An embodiment is directed to phosphorus-containing copolymer compounds having the general structure:



wherein each R is an independently selected alkylphenol-free moiety that is a  $C_{1-22}$  alkyl,  $C_{6-40}$  cycloalkyl,  $C_{3-20}$  methoxy alkyl glycol ether,  $C_{3-20}$  alkyl glycol ether, or Y—OH moiety;

wherein each Y is an independently selected alkylphenol-free moiety that is a  $C_{2-40}$  alkylene,  $C_{6-40}$  cycloalkylene,  $C_{2-20}$  alkylene glycol ether, or  $C_{3-40}$  alkylene lactone moiety; wherein  $Y_1$  and  $Y_2$  are different;

wherein each m is an independently selected integer ranging from 1 to 100;

wherein each Z is independently selected from the group consisting of S, H, O, and nothing; and

wherein each x is an independently selected integer ranging from 1 to 1000.

In some phosphorus-containing copolymer embodiments, each Y is an independently selected ethylene, propylene, cyclohexene dimethanol, or caprylene lactone moiety.

In some embodiments, each Z is independently selected from the group consisting of S, H, and O.

In some phosphorus-containing copolymer compound embodiments, the compound has a weight ranging from 1000 to 30000 Daltons. In some phosphorus-containing copolymer compound embodiments, the compound has a weight ranging from 400 to 30000 Daltons. In some phosphorus-containing copolymer compound embodiments, the compound has a weight ranging from 500 to 30000 Daltons.

An embodiment is directed to phosphite compounds having the general structure:



wherein each R is an independently selected alkylphenol-free moiety that is a  $C_{1-22}$  alkyl,  $C_{6-40}$  cycloalkyl,  $C_{3-20}$  methoxy alkyl glycol ether,  $C_{3-20}$  alkyl glycol ether, or Y—OH moiety;

wherein each Y is an independently selected alkylphenol-free moiety that is a  $C_{2-40}$  alkylene,  $C_{6-40}$  cycloalkylene,  $C_{2-20}$  alkylene glycol ether, or  $C_{3-40}$  alkylene lactone moiety; wherein each m is an independently selected integer ranging from 1 to 100; and

wherein x is an integer ranging from 1 to 1000.

In some phosphite embodiments, each Y is an independently selected ethylene, propylene, cyclohexene dimethanol, or caprylene lactone moiety.

In some phosphorus-compound embodiments, the compound has a weight ranging from 1000 to 30000 Daltons. In some phosphorus-containing copolymer compound embodiments, the compound has a weight ranging from 400 to 30000 Daltons. In some phosphorus-containing copolymer compound embodiments, the compound has a weight ranging from 500 to 30000 Daltons.

Methods for manufacturing any of the disclosed compounds that include phosphite compounds, polyhydrogen

phosphite compounds, phosphate compounds, thiophosphate compounds, and thiophosphite-phosphate copolymer compounds can be determined by persons of ordinary skill in the art without having to exercise undue experimentation. Non-limiting examples of manufacturing methods can be found in the below Examples.

Any of the above compounds, either alone or in any combination, can be used as an additive for: gear oil, grease, engine-oil, combustion-engine lubricant, automatic transmission fluid, two-cycle engine lubricant, or marine-engine lubricant. The compounds, either alone or in any combination, are also useful as anti-wear additives. For each of the described uses, useful amounts of the compound(s) can be determined by persons of ordinary skill in the art. As a non-limiting example, useful amounts of the above compounds, either alone or in any combination, range from 5 to 10% by weight of the fluid to which the compound(s) is being added. In an additional non-limiting example, useful amounts of the above compound(s), either alone or in any combination, range from 0.5 to 20% by weight of the fluid to which the compound(s) is being added.

In any of the above sulfur-containing compounds, the amount of sulfur within the compound can range from 50 to 100 mole percent relative to the amount of phosphorus within the compound; stated differently, in any of the above sulfur-containing compounds, anywhere from half to all of the phosphorus atoms are bonded to a sulfur atom. In another embodiment, the amount of sulfur within the compound can range from 90 to 100 mole percent relative to the amount of phosphorus within the compound. In another embodiment, the amount of sulfur within the compound is 100 mole percent relative to the amount of phosphorus within the compound.

Although all of the above compounds are taught as having alkylphenol-free moieties, in some embodiments, a compound's above-described alkylphenol-free moiety is replaced with an alkylphenol moiety. In other embodiments, more than one of a compound's above-described alkylphenol-free moieties is replaced with an alkylphenol moieties. Here is a non-limiting example of a compound containing an alkylphenol moiety:



wherein each R is an independently selected alkylphenol moiety or an independently selected alkylphenol-free moiety that is a C<sub>1-22</sub> alkyl, C<sub>6-40</sub> cycloalkyl, C<sub>3-20</sub> methoxy alkyl glycol ether, C<sub>3-20</sub> alkyl glycol ether, or Y—OH moiety; wherein each Y is an independently selected alkylphenol moiety or an independently selected alkylphenol-free moiety that is a C<sub>2-40</sub> alkylene, C<sub>6-40</sub> cycloalkylene, C<sub>2-20</sub> alkylene glycol ether, or C<sub>3-40</sub> alkylene lactone moiety; wherein each m is an independently selected integer ranging from 1 to 100; and wherein x is an integer ranging from 1 to 1000.

Here is another non-limiting example of a compound containing an alkylphenol moiety:



wherein each R is an independently selected alkylphenol moiety or an independently selected alkylphenol-free moiety that is a C<sub>1-22</sub> alkyl, C<sub>6-40</sub> cycloalkyl, C<sub>3-20</sub> methoxy alkyl glycol ether, C<sub>3-20</sub> alkyl glycol ether, or Y—OH moiety; wherein each Y is an independently selected alkylphenol moiety or an independently selected alkylphenol-free moiety that is a C<sub>2-40</sub> alkylene, C<sub>6-40</sub> cycloalkylene, C<sub>2-20</sub> alkylene glycol ether, or C<sub>3-40</sub> alkylene lactone moiety; wherein each m is an independently selected integer ranging from 1 to 100; and wherein x is an integer ranging from 1 to 1000.

Here is another non-limiting example of a compound containing an alkylphenol moiety:



wherein each R is an independently selected alkylphenol moiety or an independently selected alkylphenol-free moiety that is a C<sub>1-22</sub> alkyl, C<sub>6-40</sub> cycloalkyl, C<sub>3-20</sub> methoxy alkyl glycol ether, C<sub>3-20</sub> alkyl glycol ether, or Y—OH moiety; wherein each Y is an independently selected alkylphenol moiety or an independently selected alkylphenol-free moiety that is a C<sub>2-40</sub> alkylene, C<sub>6-40</sub> cycloalkylene, C<sub>2-20</sub> alkylene glycol ether, or C<sub>3-40</sub> alkylene lactone moiety; wherein each m is an independently selected integer ranging from 1 to 100; and wherein x is an integer ranging from 1 to 1000.

Here is another non-limiting example of a compound containing an alkylphenol moiety:



wherein each R is an independently selected alkylphenol moiety or an independently selected alkylphenol-free moiety that is a C<sub>1-22</sub> alkyl, C<sub>6-40</sub> cycloalkyl, C<sub>3-20</sub> methoxy alkyl glycol ether, C<sub>3-20</sub> alkyl glycol ether, or Y—OH moiety; wherein each Y is an independently selected alkylphenol moiety or an independently selected alkylphenol-free moiety that is a C<sub>2-40</sub> alkylene, C<sub>6-40</sub> cycloalkylene, C<sub>2-20</sub> alkylene glycol ether, or C<sub>3-40</sub> alkylene lactone moiety; wherein each m is an independently selected integer ranging from 1 to 100; wherein each Z is independently selected from the group consisting of S and O; and wherein x is an integer ranging from 1 to 1000.

Here is another non-limiting example of a compound containing an alkylphenol moiety:



wherein each R is an independently selected alkylphenol moiety or an independently selected alkylphenol-free moiety that is a C<sub>1-22</sub> alkyl, C<sub>6-40</sub> cycloalkyl, C<sub>3-20</sub> methoxy alkyl glycol ether, C<sub>3-20</sub> alkyl glycol ether, or Y—OH moiety; wherein each Y is an independently selected alkylphenol moiety or an independently selected alkylphenol-free moiety that is a C<sub>2-40</sub> alkylene, C<sub>6-40</sub> cycloalkylene, C<sub>2-20</sub> alkylene glycol ether, or C<sub>3-40</sub> alkylene lactone moiety; wherein each m is an independently selected integer ranging from 1 to 100; wherein each Z is independently selected from the group consisting of S and O; and wherein each x is an independently selected integer ranging from 1 to 1000.

Here is another non-limiting example of a compound containing an alkylphenol moiety:



wherein each R is an independently selected alkylphenol moiety or an independently selected alkylphenol-free moiety that is a C<sub>1-22</sub> alkyl, C<sub>6-40</sub> cycloalkyl, C<sub>3-20</sub> methoxy alkyl glycol ether, C<sub>3-20</sub> alkyl glycol ether, or Y—OH moiety; wherein each Y is an independently selected alkylphenol moiety or an independently selected alkylphenol-free moiety that is a C<sub>2-40</sub> alkylene, C<sub>6-40</sub> cycloalkylene, C<sub>2-20</sub> alkylene glycol ether, or C<sub>3-40</sub> alkylene lactone moiety; wherein each m is an independently selected integer ranging from 1 to 100; and wherein x is an integer ranging from 1 to 1000.

In an embodiment, using a compound as an additive for gear oil, grease, engine oil, combustion-engine lubricant, automatic transmission fluid, two-cycle engine lubricant, marine-engine lubricant, or anti-wear agent means adding the compound to a gear oil, grease, engine oil, combustion-engine lubricant, automatic transmission fluid, two-cycle engine lubricant, marine-engine lubricant, or anti-wear agent. In another embodiment, using a compound as an additive for gear oil, grease, engine oil, combustion-engine lubricant, automatic transmission fluid, two-cycle engine lubricant, marine-engine lubricant, or anti-wear agent means using the end composition that includes the compound as a gear oil, grease, engine oil, combustion-engine lubricant, automatic transmission fluid, two-cycle engine lubricant, marine-engine lubricant, or anti-wear agent.

### Examples I

#### TNPP-T (Trisnonylphenyl thiophosphate)

To a three-neck 250 mL flask equipped with a mechanical stirrer and purged with nitrogen was added 75.83 grams of triisnonylphenol phosphite (0.110 mol), with a total non-ylphenol content ranging from 0.05% to 0.5% with 0.1%

being the target and 0.39 grams of 2,5-dimercapto-1,3,4-thiadiazole (0.0026 mol). The mixture was mixed well and heat was applied to a reaction temperature of 240° F. 3.37 grams of elemental sulfur (0.130 mol) was then added at this temperature. After one hour, the reaction temperature is increased to 280° F. and held for 16-24 hours. This reaction takes place under a nitrogen blanket. The resulting thiophosphate had the following analysis:

|    |               |       |
|----|---------------|-------|
| 10 | % Phosphorous | 4.5   |
|    | % Sulfur      | 4.2   |
|    | Density 20 C  | 1.01  |
|    | Color, APHA   | 50    |
| 15 | % Nonylphenol | <0.20 |

LGP-11-T (Alkylphenol Free Polymeric Polyphosphite), U.S. Pat. No. 8,563,637B

To a three-neck 250 mL flask equipped with a mechanical stirrer and purged with nitrogen was added 75.83 grams of a alkylphenol-free liquid polymeric phosphite (Example #2 from U.S. Pat. No. 8,563,637), with a molecular weight of about 9100 and 0.39 grams of 2,5-dimercapto-1,3,4-thiadiazole (0.0026 mol). The mixture was mixed well and heat was applied to a reaction temperature of 240° F. Then 3.51 grams of elemental sulfur (0.109 mol) was added. After one hour, the reaction temperature is increased to 280° F. and held for 16-24 hours. This reaction takes place under a nitrogen blanket. The resulting alkyl phenol free polymeric thiophosphate had the following analysis:

|    |               |     |
|----|---------------|-----|
| 35 | % Phosphorous | 4.7 |
|    | % Sulfur      | 4.4 |
|    | Density 20 C  |     |
|    | Color, APHA   | 60  |
| 30 | % Nonylphenol | 0   |

LGP-12-T (Alkylphenol Free Cycloaliphatic Poly and Copoly Phosphites) U.S. Pat. No. 8,981,042B2

To a three-neck 250 mL flask equipped with a mechanical stirrer and purged with nitrogen was added 75.83 grams of cycloaliphatic polyphosphite (Example 2 from U.S. Pat. No. 8,981,042) with a molecular weight range of about 14,000 and 0.39 grams of 2,5-dimercapto-1,3,4-thiadiazole (0.0026 mol). The mixture was mixed well and heat was applied to a reaction temperature of 240° F. 5.52 grams of elemental sulfur (0.172 mol) was then added. After one hour, the reaction temperature is increased to 280° F. and held for 16-24 hours. This reaction takes place under a nitrogen blanket. The resulting analysis of the phenol free cycloaliphatic alkylated poly thiophosphate was:

|    |               |      |
|----|---------------|------|
| 55 | % Phosphorous | 7.2  |
|    | % Sulfur      | 6.75 |
|    | Color, APHA   | 50   |
|    | % Nonylphenol | 0    |

LGP(DPG)-11-T, U.S. Pat. No. 8,563,637B

To a three-neck 250 mL flask equipped with a mechanical stirrer and purged with nitrogen was added 75.83 grams of a alkylphenol-free liquid polymeric phosphite (Example #3 from U.S. Pat. No. 8,563,637), with a molecular weight of about 1200 and 0.39 grams of 2,5-dimercapto-1,3,4-thiadiazole (0.0026 mol). The mixture was mixed well and heat was applied to a reaction temperature of 240° F. Then 6.29 grams of elemental sulfur (0.196 mol) was added. After one

## 11

hour, the reaction temperature is increased to 280° F. and held for 16-24 hours. This reaction takes place under a nitrogen blanket. The resulting alkyl phenol free polymeric thiophosphate had the following analysis:

|               |     |
|---------------|-----|
| % Phosphorous | 7.8 |
| % Sulfur      | 7.6 |
| Color, APHA   | 60  |
| % Nonylphenol | 0   |

## DP-6T (Triisodecyl Phosphite) Doverphos 6

To a three-neck 250 mL flask equipped with a mechanical stirrer and purged with nitrogen was added 75.83 grams of a Triisodecyl phosphite, with a molecular weight of about 500 and 0.39 grams of 2,5-dimercapto-1,3,4-thiadiazole (0.0026 mol). The mixture was mixed well and heat was applied to a reaction temperature of 240° F. Then 4.87 of elemental sulfur (0.152 mol) was added. After one hour, the reaction temperature is increased to 280° F. and held for 16-24 hours. This reaction takes place under a nitrogen blanket. The resulting alkyl phenol free thiophosphate had the following analysis:

|               |     |
|---------------|-----|
| % Phosphorous | 6.2 |
| % Sulfur      | 6.0 |
| Color, APHA   | 60  |
| % Nonylphenol | 0   |

## Testing Methodology

Four Ball Wear: This test is used for evaluating friction-reducing and anti-wear fluids. Testing involves 3 stationary steel balls secured in a steel cup and a 4<sup>th</sup> steel ball lowered to make contact with the 3 stationary balls. The fluid to be tested is poured into the cup. The 4<sup>th</sup> ball is the only ball that spins. Typical rpm for the ball is 1200 rpm. The single ball spins in contact with the 3 stationary balls at a constant load of 40 kg. Typical run time is 1 hour. The wear on the lower 3 balls is measured and reported in mm. The fluid to produce the smallest wear scars has the best performance.

| Parameter     | Setting |
|---------------|---------|
| Load (kg)     | 40      |
| Temperature   | Ambient |
| Time (min)    | 60      |
| Dilution Rate | 5%      |
| Speed (rpm)   | 1,200   |

## Wear Scar (mm)

| Ball    | Example 1 | Example 2 | Example 3 | Example 4 | Example 5 |
|---------|-----------|-----------|-----------|-----------|-----------|
| 1       | 0.91      | 0.39      | 0.52      | 0.52      | 0.57      |
| 2       | 0.91      | 0.39      | 0.52      | 0.52      | 0.55      |
| 3       | 0.86      | 0.39      | 0.52      | 0.52      | 0.55      |
| Avg. mm | 0.89      | 0.39      | 0.52      | 0.52      | 0.55      |

Test results clearly show that the alkylphenol free polymeric polyphosphites give excellent results, better than the commercial trisnonylphenyl thiophosphate with excellent color. And there are no alkylphenols in the final products.

Timken Testing: Timken testing was carried out by adding weight to a lever applying pressure to a block that is in

## 12

contact with a wheel. The bottom portion of the wheel is submersed in the fluid to be tested. As the wheel spins, the lubricant is carried to the interface of the block and wheel. A one pound weight is added to the lever every minute until a maximum of 13 pounds has been added. The wear scar on the block is measured and reported in millimeters. See FIG. 1.

## Wear Scar (mm)

|    | Example 1 | Example 2 | Example 3 | Example 4 | Example 5 |
|----|-----------|-----------|-----------|-----------|-----------|
| 10 | 2.34      | 2.08      | 2.08      | 2.24      | 2.60      |

Test results clearly show that the alkylphenol free polymeric polyphosphites give excellent results, better than the commercial trisnonylphenyl thiophosphate with excellent color. And there are no alkylphenols in the final products.

## Examples II

The following formulae were prepared for various machine testing:

## Oil Based Formulae

| 30                           | Additive                       | Functionality | Conc. %<br>By Weight | Methyl<br>Ester Added |
|------------------------------|--------------------------------|---------------|----------------------|-----------------------|
| Paroil 152                   | Chlorinated Paraffin           | 5             | 7                    |                       |
| Mayfree 133                  | Phosphate Amide                | 2.6           | 4.4                  |                       |
| Doverphos 253                | Di-oleyl Hydrogen<br>Phosphite | 2.6           | 7                    |                       |
| Doverphos 53                 | Tri-lauryl Phosphite           | 2.6           | 7                    |                       |
| Doverphos 50                 | Phosphite                      | 2.6           | 7                    |                       |
| Complex Ester 5%             | Ester                          | 5             | 0                    |                       |
| Complex Ester 10%            | Ester                          | 10            | 0                    |                       |
| Complex Ester 25%            | Ester                          | 25            | 0                    |                       |
| Alkylphenol Free             | Phosphite                      | 2.6           | 7                    |                       |
| Polymeric Phosphite A        |                                |               |                      |                       |
| Alkylphenol Free             | Phosphite                      | 2.6           | 7                    |                       |
| Polymeric Phosphite B        |                                |               |                      |                       |
| Base 10SE                    | Sulfurized Ester               | 5             | 2                    |                       |
| Alkylphenol Free             | Phos & Sulfur                  | 5             | 7                    |                       |
| Polymeric<br>Thiophosphate A |                                |               |                      |                       |
| Alkylphenol Free             | Phos & Sulfur                  | 5             | 7                    |                       |
| Polymeric<br>Thiophosphate B |                                |               |                      |                       |
| ZDDP                         | Phos, Sulfur & Zinc            | 2.6           | 7                    |                       |

## Water Based Formulae

The water based formulae were prepared using a commercial semi-synthetic. The additive was added to either the Super Concentrate (SC) prior to dilution of the semi-synthetic with water, or to the concentrate after 50% dilution of the semi-synthetic with water. After the 50% dilution with water, all testing was conducted with the semi-synthetic diluted in water at 5%.

| 60               | Additive | % Added<br>to S.C. | % Added to<br>Concentrate | Final<br>Conc. % |
|------------------|----------|--------------------|---------------------------|------------------|
| Paroil 152       | 5        | 0                  | 5                         |                  |
| Mayfree 133      | 0        | 2.6                | 5                         |                  |
| Doverphos 253    | 0        | 2.6                | 5                         |                  |
| Doverphos 53     | 0        | 2.6                | 5                         |                  |
| Doverphos 50     | 0        | 2.6                | 5                         |                  |
| Complex Ester 5% | 0        | 5                  | 5                         |                  |

13

-continued

| Additive                   | % Added to S.C. | % Added to Concentrate | Final Conc. % |    |
|----------------------------|-----------------|------------------------|---------------|----|
| Alkylphenol Free Polymeric | 0               | 2.6                    | 5             | 5  |
| Phosphite A                |                 |                        |               |    |
| Alkylphenol Free Polymeric | 0               | 2.6                    | 5             | 10 |
| Phosphite B                |                 |                        |               |    |

## Testing Methodology

## Oil Based Testing:

Four Ball Wear: This test is used for evaluating friction-reducing and anti-wear fluids. Testing involves 3 stationary steel balls secured in a steel cup and a 4<sup>th</sup> steel ball lowered to make contact with the 3 stationary balls. The fluid to be tested is poured into the cup. The 4<sup>th</sup> ball is the only ball that spins. Typical rpm for the ball is 1200 rpm. The single ball spins in contact with the 3 stationary balls at a constant load of 40 kg. Typical run time is 1 hour. The wear on the lower 3 balls is measured and reported in mm. The fluid to produce the smallest wear scars has the best performance.

| Parameter   | Setting |
|-------------|---------|
| Load (kg)   | 40      |
| Temperature | Ambient |
| Time (min)  | 60      |
| Speed (rpm) | 1,200   |

## Wear Scar (mm)

| Additive                   | Average Wear, mm |
|----------------------------|------------------|
| Paroil 152, Std.           | 0.99             |
| Doverphos 53               | 0.41             |
| ZDDP                       | 0.45             |
| Base 10SE                  | 0.52             |
| Doverphos 253              | 0.54             |
| Mayfree 133                | 0.61             |
| Alkylphenol Free Polymeric | 0.36             |
| Phosphite A                |                  |
| Alkylphenol Free Polymeric | 0.49             |
| Phosphite B                |                  |
| Doverphos 50               | 0.46             |
| Alkylphenol Free Polymeric | 0.36             |
| Thiophosphate A            |                  |
| Alkylphenol Free Polymeric | 0.39             |
| Thiophosphate B            |                  |
| Polymeric Ester-5%         | 0.66             |
| Polymeric Ester-10%        | 0.65             |
| Polymeric Ester-25%        | 0.53             |

Vertical Drawbead: Vertical Drawbead is a machine used to determine a fluids ability to form a piece of metal. Vertical Drawbead works by applying pressure to a coated metal strip. The formulae to be tested is applied to a 24 inch metal strip which is raised between two dye. The dyes apply 500 psi of pressure to the bottom of the strip. The coated strip is pulled between the two dyes. The amount of force needed to pull the strip between the dyes, is plotted by an X-Y plotter and the force is calculated from this curve. In all cases, higher percent efficiency refers to the performance of the fluid being better.

In this test, all formulae were evaluated on 1018 Steel and 316 Stainless Steel.

14

316 Stainless Steel

| Additive                   | % Efficiency |
|----------------------------|--------------|
| Paroil 152, Std.           | 100.0        |
| Doverphos 53               | 95.1         |
| ZDDP                       | 103.8        |
| Base 10SE                  | 81.0         |
| Doverphos 253              | 77.3         |
| Mayfree 133                | 102.2        |
| Alkylphenol Free Polymeric | 70.3         |
| Phosphite A                |              |
| Alkylphenol Free Polymeric | 46.4         |
| Phosphite B                |              |
| Doverphos 50               | 103.8        |
| Alkylphenol Free Polymeric | 114.2        |
| Thiophosphate A            |              |
| Alkylphenol Free Polymeric | 119.0        |
| Thiophosphate B            |              |
| Polymeric Ester-5%         | 112.5        |
| Polymeric Ester-10%        | 116.8        |
| Polymeric Ester-25%        | 147.6        |

1018 Steel

| Additive                   | % Efficiency |
|----------------------------|--------------|
| Paroil 152, Std.           | 100.0        |
| Doverphos 53               | 109.4        |
| ZDDP                       | 103.8        |
| Base 10SE                  | 103.3        |
| Doverphos 253              | 105.4        |
| Mayfree 133                | 97.1         |
| Alkylphenol Free Polymeric | 103.5        |
| Phosphite A                |              |
| Alkylphenol Free Polymeric | 102.3        |
| Phosphite B                |              |
| Doverphos 50               | 111.6        |
| Alkylphenol Free Polymeric | 107.0        |
| Thiophosphate A            |              |
| Alkylphenol Free Polymeric | 102.3        |
| Thiophosphate B            |              |
| Polymeric Ester-5%         | 111.9        |
| Polymeric Ester-10%        | 113.1        |
| Polymeric Ester-25%        | 129.5        |

Microtap Tap and Torque Testing: Microtap testing is one method used to determine a fluids ability to remove metal. A metal bar with predrilled holes is fastened to a vice. The tap and the metal bar are coated in the fluid to be tested. The tap rotates to tap out the pre-drilled hole. The force needed to tap the hole is measured by a computer and is reported as torque in newton centimeters. In all cases, higher percent efficiency refers to the performance of the fluid being better.

In this test, all formulae were evaluated on 1018 Steel.

1018 Steel

| Additive                   | % Efficiency |
|----------------------------|--------------|
| Paroil 152, Std.           | 100.0        |
| Doverphos 53               | 101.7        |
| ZDDP                       | 101.1        |
| Base 10SE                  | 100.5        |
| Doverphos 253              | 101.1        |
| Mayfree 133                | 103.8        |
| Alkylphenol Free Polymeric | 103.1        |
| Phosphite A                |              |
| Alkylphenol Free Polymeric | 102.9        |
| Phosphite B                |              |
| Doverphos 50               | 103.8        |
| Alkylphenol Free Polymeric | 103.5        |
| Thiophosphate A            |              |
| Alkylphenol Free Polymeric | 104.3        |

## 15

-continued

| Additive            | % Efficiency |
|---------------------|--------------|
| Thiophosphate B     |              |
| Polymeric Ester-5%  | 105.2        |
| Polymeric Ester-10% | 104.0        |
| Polymeric Ester-25% | 106.9        |

Falex Pin and Vee Block Testing: Falex Pin and Vee Block measures the fluids ability to perform in more severe operations, such as cold heading, but can also apply to grinding operations. A pin is fastened using a brass shear pin. Two Vee blocks are clamped onto the pin. The pin and vee blocks are submerged in the fluid to be tested. The load applied on the pin from the vee blocks begins at 250 pounds. The load is increased automatically by a ratcheting arm as the pin spins between the two vee blocks. The torque generated by the load on the pin is read at 250 pound load and is recorded every 250 pounds until a final load of 4500 pounds is reached or a failure occurs. A failure implies the pin or shear pin has broken. See FIGS. 2 and 3.

## Water Based Testing:

Microtap Tap and Torque Testing: Microtap testing is one method used to determine a fluids ability to remove metal. A metal bar with predrilled holes is fastened to a vice. The tap and the metal bar are coated in the fluid to be tested. The tap rotates to tap out the predrilled hole. The force needed to tap the hole is measured by a computer and is reported as torque in newton centimeters. In all cases, higher percent efficiency refers to the performance of the fluid being better.

In this test, all formulae were evaluated on 1018 Steel and 316 Stainless Steel.

## 316 Stainless Steel

| Additive                               | % Efficiency |
|----------------------------------------|--------------|
| Paroil 152, Std.                       | 100.0        |
| Doverphos 53                           | 108.6        |
| Doverphos 253                          | 112.0        |
| Mayfree 133                            | 117.6        |
| Alkylphenol Free Polymeric Phosphite A | 109.4        |
| Alkylphenol Free Polymeric Phosphite B | 112.1        |
| Doverphos 50                           | 109.4        |
| Polymeric Ester-5%                     | 107.6        |

## 1018 Steel

| Additive                               | % Efficiency |
|----------------------------------------|--------------|
| Paroil 152, Std.                       | 100.0        |
| Doverphos 53                           | 102.4        |
| Doverphos 253                          | 101.1        |
| Mayfree 133                            | 101.9        |
| Alkylphenol Free Polymeric Phosphite A | 100.9        |
| Alkylphenol Free Polymeric Phosphite B | 100.2        |
| Doverphos 50                           | 100.0        |
| Polymeric Ester-5%                     | 99.3         |

Falex Pin and Vee Block Testing: Falex Pin and Vee Block measures the fluids ability to perform in more severe operations, such as cold heading, but can also apply to grinding operations. A pin is fastened using a brass shear pin. Two Vee blocks are clamped onto the pin. The pin and vee blocks are submerged in the fluid to be tested. The load applied on

## 16

the pin from the vee blocks begins at 250 pounds. The load is increased automatically by a ratcheting arm as the pin spins between the two vee blocks. The torque generated by the load on the pin is read at 250 pound load and is recorded every 250 pounds until a final load of 4500 pounds is reached or a failure occurs. A failure implies the pin or shear pin has broken. See FIGS. 4 and 5.

10 What is claimed is:

1. A method comprising the step:

adding a compound in an amount ranging from 0.5% to 10% by weight to: gear oil, grease, engine oil, combustion-engine lubricant, automatic transmission fluid, two-cycle engine lubricant, marine-engine lubricant, or anti-wear agent; to thereby improve the respective anti-wear properties, the compound having the structure:



wherein each R is an independently selected alkylphenol-free moiety that is a  $\text{C}_{1-6}$  alkyl moiety,  $\text{C}_6$  cycloalkyl moiety, or Y—OH moiety;

30 wherein each Y is an independently selected alkylphenol-free moiety that is a  $\text{C}_{2-40}$  alkylene moiety,  $\text{C}_{6-40}$  cycloalkylene moiety,  $\text{C}_{2-20}$  alkylene glycol ether moiety, or  $\text{C}_{3-40}$  alkylene lactone moiety;

35 wherein each m is an independently selected integer ranging from 1 to 100; and

wherein x is an integer ranging from 1 to 1000.

2. The method of claim 1, wherein each Y is an independently selected ethylene moiety, propylene moiety, cyclohexene dimethanol moiety, or caprylene lactone moiety.

3. The method of claim 1, wherein the compound has a weight ranging from 1000 to 30000 Daltons.

4. The method of claim 1, wherein the compound has a weight ranging from 400 to 30000 Daltons.

45 5. The method of claim 1, wherein the compound has a weight ranging from 500 to 30000 Daltons.

6. A method comprising the step:  
adding a compound to: gear oil, grease, engine oil, combustion-engine lubricant, automatic transmission fluid, two-cycle engine lubricant, marine-engine lubricant, or anti-wear agent; to thereby improve the respective anti-wear properties, the compound having the structure:



65 wherein each R is an independently selected alkylphenol-free moiety that is a  $\text{C}_{1-22}$  alkyl moiety,  $\text{C}_{6-40}$  cycloalkyl moiety,  $\text{C}_{3-20}$  methoxy alkyl glycol ether moiety,  $\text{C}_{3-20}$  alkyl glycol ether moiety, or Y—OH moiety;

17

wherein each Y is an independently selected alkylphenol-free moiety that is a  $C_{2-40}$  alkylene moiety,  $C_{6-40}$  cycloalkylene moiety,  $C_{2-20}$  alkylene glycol ether moiety, or  $C_{3-40}$  alkylene lactone moiety;

wherein each m is an independently selected integer ranging from 2 to 100; and

wherein x is an integer ranging from 1 to 1000.

7. The method of claim 6, wherein each Y is an independently selected ethylene moiety, propylene moiety, cyclohexene dimethanol moiety, or caprylene lactone moiety.

8. The method of claim 6, wherein the compound has a weight ranging from 1000 to 30000 Daltons.

9. The method of claim 6, wherein the compound has a weight ranging from 400 to 30000 Daltons.

10. The method of claim 6, wherein the compound has a weight ranging from 500 to 30000 Daltons.

**11. A method comprising the step:**

adding a compound to: gear oil, grease, engine oil, combustion-engine lubricant, automatic transmission fluid, two-cycle engine lubricant, marine-engine lubricant, or anti-wear agent; to thereby improve the respective anti-wear properties, the compound having the structure:



wherein each R is an independently selected alkylphenol-free moiety that is a  $C_{1-22}$  alkyl moiety,  $C_{6-40}$  cycloalkyl moiety,  $C_{3-20}$  methoxy alkyl glycol ether moiety,  $C_{3-20}$  alkyl glycol ether moiety, or Y—OH moiety;

wherein each Y is an independently selected alkylphenol-free moiety that is a  $C_{2-40}$  alkylene moiety,  $C_{6-40}$  cycloalkylene moiety,  $C_{2-20}$  alkylene glycol ether moiety, or  $C_{3-40}$  alkylene lactone moiety;

wherein each m is an independently selected integer ranging from 2 to 100; and

wherein x is an integer ranging from 1 to 1000.

12. The method of claim 11, wherein each Y is an independently selected ethylene moiety, propylene moiety, cyclohexene dimethanol moiety, or caprylene lactone moiety.

13. The method of claim 11, wherein the compound has a weight ranging from 1000 to 30000 Daltons.

14. The method of claim 11, wherein the compound has a weight ranging from 400 to 30000 Daltons.

15. The method of claim 11, wherein the compound has a weight ranging from 500 to 30000 Daltons.

**16. A method comprising the step:**

adding a compound to: gear oil, grease, engine oil, combustion-engine lubricant, automatic transmission fluid, two-cycle engine lubricant, marine-engine lubricant, or anti-wear agent; to thereby improve the respective anti-wear properties, the compound having the structure:

18



10 wherein each R is an independently selected alkylphenol-free moiety that is a  $C_{1-22}$  alkyl moiety,  $C_{6-40}$  cycloalkyl moiety,  $C_{3-20}$  methoxy alkyl glycol ether moiety,  $C_{3-20}$  alkyl glycol ether moiety, or Y—OH moiety;

wherein each Y is an independently selected alkylphenol-free moiety that is a  $C_{2-40}$  alkylene moiety,  $C_{6-40}$  cycloalkylene moiety,  $C_{2-20}$  alkylene glycol ether moiety, or  $C_{3-40}$  alkylene lactone moiety;

wherein each m is an independently selected integer ranging from 2 to 100;

wherein each Z is independently selected from the group consisting of S and O; and

wherein x is an integer ranging from 1 to 1000.

15 17. The method of claim 16, wherein each Y is an independently selected ethylene moiety, propylene moiety, cyclohexene dimethanol moiety, or caprylene lactone moiety.

20 18. The method of claim 16, wherein the compound has a weight ranging from 1000 to 30000 Daltons.

19. The method of claim 16, wherein the compound has a weight ranging from 400 to 30000 Daltons.

20 20. The method of claim 16, wherein the compound has a weight ranging from 500 to 30000 Daltons.

**21. A method comprising the step:**

adding a compound to: gear oil, grease, engine oil, combustion-engine lubricant, automatic transmission fluid, two-cycle engine lubricant, marine-engine lubricant, or anti-wear agent; to thereby improve the respective anti-wear properties, the compound having the structure:



40 wherein each R is an independently selected alkylphenol-free moiety that is a  $C_{1-22}$  alkyl moiety,  $C_{6-40}$  cycloalkyl moiety,  $C_{3-20}$  methoxy alkyl glycol ether moiety,  $C_{3-20}$  alkyl glycol ether moiety, or Y—OH moiety;

50 wherein each Y is an independently selected alkylphenol-free moiety that is a  $C_{2-40}$  alkylene moiety,  $C_{6-40}$  cycloalkylene moiety,  $C_{2-20}$  alkylene glycol ether moiety, or  $C_{3-40}$  alkylene lactone moiety;

55 wherein  $Y_1$  and  $Y_2$  are different;

wherein each m is an independently selected integer ranging from 1 to 100;

wherein  $m_1+m_2=3$  or more;

60 wherein each Z is independently selected from the group consisting of S, H, O, and nothing; and

wherein each x is an independently selected integer ranging from 1 to 1000.

65 22. The method of claim 21, wherein each Y is an independently selected ethylene moiety, propylene moiety, cyclohexene dimethanol moiety, or caprylene lactone moiety.

## 19

23. The method of claim 21, wherein the compound has a weight ranging from 1000 to 30000 Daltons.
24. The method of claim 21, wherein the compound has a weight ranging from 400 to 30000 Daltons.
25. The method of claim 21, wherein the compound has a weight ranging from 500 to 30000 Daltons.
26. A method comprising the step:

adding a compound to: gear oil, grease, engine oil, combustion-engine lubricant, automatic transmission fluid, two-cycle engine lubricant, marine-engine lubricant, or anti-wear agent; to thereby improve the respective anti-wear properties, the compound having the structure:



wherein each R is an independently selected alkylphenol-free moiety that is a  $C_{6-40}$  cycloalkyl moiety,  $C_{3-20}$  methoxy alkyl glycol ether moiety,  $C_{3-20}$  alkyl glycol ether moiety, or Y—OH moiety;

## 20

- wherein each Y is an independently selected alkylphenol-free moiety that is a  $C_{2-40}$  alkylene moiety,  $C_{6-40}$  cycloalkylene moiety,  $C_{2-20}$  alkylene glycol ether moiety, or  $C_{3-40}$  alkylene lactone moiety;
- 5 wherein each m is an independently selected integer that is 2 or more; and
- wherein x is an integer ranging from 1 to 1000.
27. The method of claim 26, wherein each Y is an independently selected ethylene moiety, propylene moiety, cyclohexene dimethanol moiety, or caprylene lactone moiety.
28. The method of claim 26, wherein the compound has a weight ranging from 1000 to 30000 Daltons.
29. The method of claim 26, wherein the compound has a weight ranging from 400 to 30000 Daltons.
- 10 30. The method of claim 26, wherein the compound has a weight ranging from 500 to 30000 Daltons.
31. The method of claim 21, wherein each Z is independently selected from the group consisting of S, H, and O.
- 20 32. The method of claim 1, wherein the compound is added in an amount ranging from 5% to 10% by weight.
33. The method of claim 1, wherein the compound is added in an amount of about 2.6% by weight.
- 25 34. The method of claim 1, wherein the compound is added in an amount ranging from 0.5% by weight to 2.6% by weight.

\* \* \* \* \*